

July 13, 1965

W. A. BIGGS, JR., ETAL

3,194,275

SPIRALLY WOUND PAPER TUBE

Filed Jan. 15, 1963

2 Sheets-Sheet 1

H1G-1

H1G-2



INVENTORS:  
WILLIAM A. BIGGS, JR. and  
CHARLES K. DUNLAP, JR.  
BY

Russell Foster

July 13, 1965

W. A. BIGGS, JR., ETAL

3,194,275

SPIRALLY WOUND PAPER TUBE

Filed Jan. 15, 1963

2 Sheets-Sheet 2



FIG-3



FIG-4



FIG-5

3,194,275

**SPIRALLY WOUND PAPER TUBE**

William A. Biggs, Jr., and Charles K. Dunlap, Jr., Hartsville, S.C., assignors to Sonoco Products Company, Hartsville, S.C., a corporation of South Carolina

Filed Jan. 15, 1963, Ser. No. 251,614

3 Claims. (Cl. 138—144)

This invention relates to paper tubes and more particularly to a spirally wound paper tube for the winding of sheet material such as textile material and the like.

It is a common practice today to utilize wound, multiply paper tubes as carriers or cores for sheet material such as paper, cloth, carpet material and the like. Such tubes or cores used for the winding of heavy sheet material such as carpet material are required to be of high strength to resist crushing and buckling when subjected to the forces generally encountered when wound with such carpet material and the like. Carpet material is generally wound in long lengths on its tubular carrier producing a very heavy load and although the spiral tube of the invention may be used for the winding of any material where a strong carrier is desired, it is particularly useful for the winding of such heavy carpet material.

Paper tubes in use today as a carrier for long lengths of carpet material are required to have both a high resistance to radial crushing and a high beam strength which, as is well known, is measured by the ability of the tube to withstand a centrally positioned load with the tube supported only at its ends. Such present day tubes or cores are generally made by convolutely winding a paper web into a tube as a convolutely wound tube has by its nature a beam strength greatly in excess of a spirally wound tube together with a satisfactory degree of crush strength. Furthermore, the convolute tube when subjected to a beam load fails by a buckling or pleating of its walls whereas the spiral tube fails by splitting along its spiral tube seam or what is known as "seam splitting." Such seam splitting is highly undesirable in that it pinches the material wound on the core with resulting damage to the material.

Primarily because of its lower cost of production, there has been a continuous search for a spiral tube which will provide the beam and crush strength of the convolutely wound tube for use in such areas of use as described above. While spirally wound tubes have been well known from the earliest times, a suitable spiral tube for such a use has not heretofore been obtained. In addition to the high radial crushing strength of spiral tubes in comparison with convolute tubes, their uniform concentricity and radial dimensional stability, the low production costs common to the spiral tube has intensified the search all to no avail. Some progress has been made in increasing the beam strength of such spiral tubes by increasing the wall thickness of the tube and with the use of stronger paper but the resulting tubes still have far less than the desired strength and the slight strength increase obtained is offset by the high cost and increased bulkiness of the tubes.

Accordingly, a primary object of this invention is to provide a new and novel spiral tube having a high beam strength and high crush strength.

Another object of this invention is to provide a new and novel spiral tube for use as a core or carrier for heavy sheet material such as carpet material and the like.

A further object of this invention is to provide a new and novel spiral tube for use as a core for heavy sheet material which tube has a beam strength and crush strength substantially the same as a corresponding convolutely wound tube and which fails by buckling rather than by seam splitting so as to avoid damage to the material wound on the tube.

Still another object of this invention is to provide a

new and novel spiral tube having a high degree of dimensional stability so as to remain substantially constant in length throughout changes in moisture content.

This invention further contemplates the provision of a new and novel spiral tube wound at a winding angle not heretofore considered possible which is characterized by a beam strength and crush strength substantially equivalent to that of a corresponding convolutely wound tube, which utilizes spiral tube winding equipment presently available and which may be manufactured from readily available inexpensive materials at a relatively low production cost.

Other objects and advantages of the invention will become apparent from the following description taken in connection with the accompanying drawings.

In general, the objects of the invention and related objects are accomplished by providing a plurality of strips of paper which are spirally wound in overlapping relationship with adhesive therebetween to form a spiral tube.

The paper strips which contain fibers common to paper have the fibers extending lengthwise in the direction of the longitudinal axis of the paper strips or what is generally referred to as the "paper machine direction." The winding angle of the paper strips is within the range of between 15 to 27 degrees and preferably an angle of approximately 17 degrees so that the long axis of the strips and consequently the fibers in the strips approach closely a parallel relationship with the axis of the tube to provide a tube of high beam strength and high crush strength together with a high degree of dimensional stability.

The novel features which are believed to be characteristic of the invention are set forth with particularity in the appended claims. The invention itself, however, both as to its organization and method of operation may be best understood by reference to the following description taken in conjunction with the accompanying drawings in which:

FIGURE 1 is a plan view of a spiral tube winding apparatus illustrating the winding of the tube of the invention;

FIGURE 2 is a side view of a tube constructed in accordance with the invention;

FIGURE 3 is a graph illustrating the relationship between tube beam and crush strength and tube winding angle;

FIGURE 4 is a graph illustrating the relationship between the ratio of tube beam and crush strength with tube winding angle; and

FIGURE 5 is a graph illustrating the relationship between tube length change under varying moisture conditions with tube winding angle.

Referring now to the drawings and to FIGURES 1, 2 in particular, there is shown in FIGURE 2 a spiral tube designated generally by the letter T which is constructed in accordance with the invention. The spiral tube T is wound on slightly modified conventional spiral tube winding apparatus portions of which are shown in FIGURE 1. The apparatus of FIGURE 1 includes a frame designated generally by the numeral 11 arranged to support a winding mandrel 12 around which a continuous belt 13 is looped in the conventional manner for advancing the tube T in the direction of the arrow P. The belt 13 is mounted in the conventional manner on drums or pulleys 14, 16 at least one of which is rotatable by suitable driving means and the pulleys 14, 16 are arranged for adjustable sliding movement on a frame 17 positioned for angular adjustment on a base 18. The spacing between the drums 14, 16 is adjusted by means of threaded shafts 19, 20 arranged to be manually rotated by means of hand wheels 21, 22 respectively for belt tensioning purposes.

The spiral tube T of the invention is wound from a plurality of plies or strips of paper containing fibers common to paper and, in the specific embodiment illustrated, the

paper strips are seven in number including an inner strip 23, intermediate strips 24, 25, 26, 27, 28 and outer strip 29. The paper strips 23 through 29 are formed in a conventional manner on a paper making machine but all of the strips employed in the construction of the tube T of the invention are made by the well-known technique wherein the fibers of the strips lie substantially parallel with the longitudinal axis of the strips or in the direction of the arrows I. In other words, the paper strips 23 to 29 have their longitudinal axis parallel to what is referred to as the "paper making machine direction." This is accomplished by cutting the paper web parallel to the direction the web travels during its formation on the paper machine to form the strips 23-29.

In the manufacture of spiral tubes under present day practice, the winding angle, identified in FIGURES 1, 2 as  $X^\circ$ , is generally within the range of 50 to 80 degrees and as has been explained tubes made at a winding angle within this range do not have the desired beam strength. In accordance with the invention, the winding angle  $X^\circ$  at which the strips 23 to 29 are wound on the winding mandrel 12 is within the range of 15 to 27 degrees preferably within the range of 17 to 22 degrees. In the specific embodiment illustrated, the winding angle  $X^\circ$  is approximately 17 degrees as it has been found that an angle of approximately 17 degrees produces the novel high strength characteristic desired in the tube T. This high strength is expressed as a beam strength to crush strength ratio as shown in the graph of FIGURE 4 and as will be explained hereinafter.

As shown in FIGURE 1, the inner paper strip 23 which forms the inner ply of the tube is wound on the mandrel 12 being brought in from one side of the spiral tube winding machine and has a suitable lubricant applied thereto by a suitable lubricating device 31. Paper strips 24 through 27 which are preferably wound onto the mandrel from the side opposite the inner strip 23 as shown are immersed in a glue bath contained in a glue pot 32 which is provided with scrapers 33 for removing excess glue from the strips as shown in FIGURE 1. Glue is not applied to the intermediate strip 28 and it is brought in dry over a set of guide rolls 34.

The top paper strip 29 is brought in from the same side of the mandrel as the intermediate strips and is advanced over a glue applicator 36. Strip 29 is then wound together with the other strips on the mandrel below the belt 13 as shown. Suitable support rollers 37 are provided on the spiral tube winder as shown in FIGURE 1 which not only aid in compressing the wound paper strips together for increased adherence but additionally serve to prevent the mandrel 12 from moving out of alignment as a result of the winding forces exerted by the belt 13 on the mandrel.

The paper strips 23 through 29 therefore form the tube T having a multi-ply side wall 38 and on its outer surface, a spiral seam 39 which as a result of the selected winding angle  $X^\circ$  lies at an angle of approximately 17 degrees relative to the longitudinal axis of the tube as shown in FIGURE 2.

The novel results accomplished with the spiral tube of the invention are shown clearly in FIGURES 3-5 and in Table I below:

TABLE I

| Paper Strip Width (inches) | Winding Angle (degrees) | Crush Strength (lbs.) | Beam Strength (lbs.) | Beam Strength/Crush Strength Ratio |
|----------------------------|-------------------------|-----------------------|----------------------|------------------------------------|
| 7 1/2-----                 | 37 1/4                  | 70                    | 281                  | 3.55                               |
| 8-----                     | 32                      | 79                    | 310                  | 3.93                               |
| 8 1/4-----                 | 29                      | 73                    | 325                  | 4.45                               |
| 8 1/2-----                 | 25 1/2                  | 64                    | 349                  | 5.45                               |
| 8 3/4-----                 | 21 1/4                  | 69                    | 382                  | 5.54                               |
| 9-----                     | 17 1/4                  | 70                    | 400                  | 5.70                               |

The results shown in Table I were obtained by winding multi-ply spiral tubes having a 3" inner diameter and a 0.150" wall thickness at winding angles ranging from a maximum of 37 1/4° to a minimum of 17 1/4°. The paper strip widths, of course, vary in accordance with the winding angle. The physical limitations of the spiral tube winding machine would not permit the winding angle to be reduced below approximately 15 degrees as at this point the length of the winding belt and the spacing of the belt drums for winding a tube at this winding angle became prohibitively large. In addition to the beam strength test as described above, a crush strength test was conducted on specimens of these various tubes both of which tests are considered in the industry as standard. As is well known, the crush strength test is carried out by loading a standard 3" length of tube between flat platens until failure.

The results of the beam strength and crush tests are tabulated in Table I and are plotted on the graph shown in FIGURE 3. It will be noted that throughout the winding angle range of approximately 37 to 17 degrees there was a 43% increase in beam strength with an accompanying crush strength decrease with only about 12%.

A ratio of beam strength to crush strength was utilized as representative of both of the desirable strength factors in a tube of the invention and FIGURE 4 shows the various ratios plotted on a graph. As explained above, the last beam strength to crush strength ratio obtained was at the 17 degree angle approximately as the physical limitations of the spiral tube winding machine militates against the winding of spiral tubes to any substantial degree below this winding angle. Points A and B plotted at the zero winding angle position of the graph of FIGURE 4 are strength ratio figures for two convoluted wound tubes of the same diameter and wall thickness on which the same tests were run and the strength ratios obtained can be considered to be those corresponding to a theoretical spiral tube having a zero degree winding angle.

It will be noted that throughout the winding angle range of approximately 17 to 27 degrees the beam strength/crush strength ratio was substantially the same and approaches substantially that of the convolute tube samples A and B. The beam strength/crush strength ratio dropped off sharply above a winding angle of approximately 27 degrees and has been explained above, a winding angle below approximately 17 degrees could not for all practical purposes be measured. It will also be noted that the beam strength/crush strength ratio of the tubes appeared to be at a maximum at a winding angle of between 17 and 22 degrees.

In addition to the high strength characteristics obtained at the low winding angles of the tubes of the invention, it was noted that the seam splitting upon failure common to spirally wound tubes subjected to a beam test did not occur but rather that the tube buckled as in the convoluted wound tube thereby avoiding the possibility of injury to material wound on the tube. This is considered to be a completely new and unexpected result and considerably enhances the commercial appeal of the tubes.

The novel results of the invention are believed to be obtained as a result of the close approach of the fibers in the paper strips used to wind the tube T to a parallel relationship with the longitudinal axis of the tube T. As a result of this positioning of the fibers of the strips forming the tube, a high resistance is offered to collapse of the tube under a beam load such as the beam strength of a convoluted wound tube which is wound with the fibers extending transversely of the "cross wound" paper sheet or, in other words, parallel to the longitudinal axis of the convolute tube. The tube T of the invention can be said to have strength characteristics closely approximating those of a convoluted wound tube.

Other new and unexpected results developed when spirally wound paper tubes wound at low winding angles

in accordance with the invention were subjected to dimensional stability tests. In conducting one such dimensional stability test on the tubes of the invention, six spiral tubes having an inner diameter of 3", a 0.150" wall thickness and a length of 30" were wound at winding angles of 36°16'; 31°55'; 28°54'; 25°36'; 21°49'; and 17°16' using seven plies of paper. In the test, the moisture content of these tubes was changed from 6% to 25% as the change in tube length resulting from this moisture content change was measured.

The resulting percent changes in length of these tubes are plotted on the graph of FIGURE 5 and it will be noted that the percent change in tube length varies from a figure of 0.82 at the higher tube winding angle of 37°16' to a percent change in length figure of 0.47 at the lower winding angle of 17°16'. Here again as in the beam strength/crush strength ratio graph the reduction in the percent change in tube length becomes increasingly small as the tube winding angle falls within the 15 to 27 degree range so that, as shown in FIGURE 5, a curve drawn through the plotted points indicates a gradual decrease in curve slope at these lower tube winding angles.

Point C in the graph of FIGURE 5 indicates the percent change in length under the same moisture content change specified above in a spirally wound tube having an inner diameter of 3 1/8", an outer diameter of 4" and a length of 30" but wound at a winding angle of 59 degrees. It will be noted that the length change with moisture content change at the higher winding angle far exceeds that of the winding angle range of the invention. The graph of FIGURE 5 thus reveals clearly that a substantial increase in dimensional stability is obtained at the lower angles of wind and the maximum dimensional stability is obtained within the range of winding angles comprising the invention.

It can be seen with the novel construction of this invention that a multi-ply spirally wound paper tube wound at winding angles not heretofore considered possible or contemplated produces completely new and unexpected results in that a spiral tube is provided having strength characteristics heretofore unobtainable in a spiral tube and obtainable only with a convolutely wound paper tube. This strength increase in the tube of the invention does not require an increase in paper nor in paper strength but is due primarily to the unusually low tube winding angle together with the use of paper strips having their fibers oriented so as to approach closely a parallel relationship with the longitudinal axis of a tube wound therefrom. The range of winding angles contemplated by the invention appear to provide the maximum strength improvement desired for spiral tubes and at the same time are within the practical considerations involved in the manufacture of such tubes.

Not only does the low angle of wind spiral tube of the invention have improved strength characteristics but seam splitting common to spiral tubes occurring upon tube

failure which is generally injurious to material wound thereon is eliminated and the tube buckles in the nature of a convolute tube. Furthermore, unusually high dimensional stability is obtained in the spiral tube of the invention in that changes in moisture content produce only very small length changes far less than those common to spiral tubes wound at the higher winding angles considerably widening the application for such spiral tubes wherein length changes must be held to a minimum.

10 While there has been described what at present is considered to be the preferred embodiment of the invention, it will be understood by those skilled in the art that various changes and modifications may be made therein without departing from the invention and, therefore, it is the 15 aim of the appended claims to cover all such changes and modifications as fall within the true spirit and scope of the invention.

Having thus described the invention, what is claimed is:

1. A spirally wound paper tube comprising, a plurality 20 of fiber containing paper strips spirally wound in overlapping relationship with adhesive therebetween to form a spiral tube, each of said paper strips having its fibers lying generally in the direction of the longitudinal axis of said strips, said strips being wound at a winding angle 25 of between about 15 to 25 degrees thereby providing a dimensionally stable tube of high beam strength and crush strength.

2. A spirally wound paper tube comprising, a plurality 30 of fiber containing paper strips spirally wound in overlapping relationship with adhesive therebetween to form a spiral tube, each of said paper strips having its fibers lying generally in the direction of the longitudinal axis of said strips, said strips being wound at a winding angle 35 of between 17 to 22 degrees thereby providing a dimensionally stable tube of high beam strength and crush strength.

3. A spirally wound paper tube comprising, a plurality 40 of fiber containing paper strips spirally wound in overlapping relationship with adhesive therebetween to form a spiral tube, each of said paper strips having its fibers lying generally in the direction of the longitudinal axis of said strips, said strips being wound at a winding angle of approximately 17 degrees thereby providing a dimensionally stable tube of high beam and crush strength.

45

#### References Cited by the Examiner

##### UNITED STATES PATENTS

|              |       |               |           |
|--------------|-------|---------------|-----------|
| 441,846      | 12/90 | Hurlbut       | 138—144   |
| 50 2,747,616 | 5/56  | De Ganahl     | 138—130 X |
| 2,749,643    | 6/56  | Scott         | 138—129 X |
| 2,825,364    | 3/58  | Cullen et al. | 138—130 X |
| 3,004,585    | 10/61 | Lewis et al.  | 138—150 X |

55 LAVERNE D. GEIGER, Primary Examiner.

LEWIS J. LENNY, Examiner.